

May 21, 1935.

J. MAZER

2,001,916

SOUND ABSORBING MATERIAL

Filed July 23, 1929

*Fig. 1.*



*Fig. 2.*



*Fig. 3.*



*Fig. 4.*



*Fig. 6. Fig. 7.*



*Fig. 5.*

INVENTOR  
Jacob Mazer,  
By Archibald Martin,  
Attorney.

## UNITED STATES PATENT OFFICE

2,001,916

## SOUND ABSORBING MATERIAL

Jacob Mazer, Stonehurst, Pa.

Application July 23, 1929, Serial No. 380,328

3 Claims. (Cl. 154—44)

My invention relates to sound-absorbing material and a method of making the same, and more particularly to materials such as are employed in the walls and ceilings of auditoriums, studios, etc., for definitely absorbing and controlling reverberation of sound waves.

Various plans have heretofore been adopted for controlling and absorbing sound waves, such as porous masonry materials, fibrous bodies, rigid cellular panels, etc.

These various materials have been open to objections such as the necessity of forming them at the place of installation, and in conjunction with the walls or ceilings to be covered, as in the case of plastic or masonry materials; the fragile nature of the fibrous bodies which are readily subject to damage through handling and which are subject to natural limitations by reason of the elasticity, size, etc., of various vegetable fibers, hair, etc., and the difficulty of applying pre-formed cellular units to spaces of various areas and contours.

One object of my invention is to provide sound-absorbing material which is highly elastic and flexible, so that it will yield under slight impacts such as those of sound waves, and which can be handled without damage and readily compressed or expanded to snugly fill designated wall spaces.

Another object of my invention is to provide a porous sound-absorbing body or unit having intercommunicating pores of desired sizes and wherein the walls of the pores are elastic.

Still another object of my invention is to provide a sound-absorbing unit whose exposed surface may be given a decorative or protective facing.

A further object of my invention is to provide a sound-absorbing body that is of generally improved characteristics in the way not only of sound-absorption, but which is simple of manufacture and conveniently handled and installed.

In the accompanying drawing, Figure 1 represents a face view of a portion of a sound-absorbing unit constructed according to my invention; Fig. 2 is a sectional view thereof; Fig. 3 shows a modification of the structure of Fig. 2; Fig. 4 shows still another modification thereof; Fig. 5 is a view, on a greatly enlarged scale, showing more clearly the cellular structure of the units, and Figs. 6 and 7 are face and edge views, respectively, showing a further modification.

Material which I employ is of a sponge-like nature containing throughout the mass cells of desired sizes, depending upon the prevailing pitches of sounds to be absorbed at a given loca-

tion. Thus, for sounds of comparatively low pitch, such as those in the neighborhood of the first octave of the musical scale (64 vibrations per second), cells of a given size will be effective in the absorption of those sounds, while in the neighborhood of the higher octaves of the musical scale, the fifth, sixth and seventh (1024, 2048 and 4096 vibrations per second, respectively), for example, cells of smaller size will be employed.

One composition of which my sound units may be formed consists of an ordinary rubber compound containing sufficient sulphur to effect vulcanization thereof in the usual manner. With this compound, I incorporate materials which may form cells in the rubber either by dissolving away portions of the rubber or by forming gases therein which will expand under heat and about which the rubber will become set upon vulcanization of the mass.

As one example of pore-forming ingredients, I may employ vegetable matter which contains moisture or which will form gases upon the application of heat below temperatures at which vulcanization is effected. For instance, wet sawdust or charcoal particles may be incorporated with the rubber. The size of the cells will be determined by the size of the gas-forming or steam-forming particles. For example, sawdust and vegetable matter which is passed through a 20 mesh screen will form larger cells than those particles of sufficient fineness to pass through a 50 mesh screen. In those cases wherein a generally inclusive sound-absorbing quality is desired, without special consideration of either the low pitch sounds or the high pitch sounds, I will incorporate gas-forming particles of various sizes. If the material is intended for use more particularly in the absorption of sounds of high pitch, I will, of course, employ finer gas-forming particles.

Other materials which when mixed with the pulverized rubber will produce pores are ammonium carbonate, soda, etc., these substances forming gases when heated to comparatively low temperatures. When the mixture containing the gas-forming particles has been brought to a temperature at which the gases are produced, it is vulcanized, thus resulting in a unit of sponge texture having the sound-absorbing and general physical characteristics above set forth, and may have the appearance of the structure shown in Figs. 1 and 2. Hydrocarbon substances, such as paraffin may also be employed.

Instead of producing a body having only cells of a given size, or having cells of large and small

sizes in intermingled relation, I may incorporate in one part of the rubber compound large gas-forming particles and in another part thereof small gas-forming particles to produce a body as shown in Fig. 3, having large cells 6 at one side thereof and small cells 7 in another portion thereof. Ordinarily, the unit of Fig. 3 would be placed on a wall or ceiling with the smaller cells outermost, so that the sounds of higher pitch will be more readily absorbed by the body, while the sounds of lower pitch will be absorbed more completely within the portion 6 of the unit than would be possible by a unit containing only the small cells.

Again, the unit may have a smooth facing 8 of rubber, paint, or other plastic material. In the case of a rubber facing, this facing could be either glued to the cellular body or vulcanized thereto. Again, if the body is vulcanized in a close-fitting mold, there will be a tendency for a skin to be formed on the surface of the article where the rubber contacts with the mold sides, thus producing a smooth exterior.

Another mixture which may be employed instead of rubber may consist of glue, glycerine, and glucose, as a base, and containing gas-generating material such as soda or some of the other materials above-enumerated. This mixture may contain from 50 to 70 pounds of softened glue, 20 to 30 pounds of glycerine, and 15 to 25 pounds of glucose, the amount of gas-generating material being of course dependent upon the extent of porosity desired in the completed body.

The body is prepared by mixing the glue, glycerine and glucose at temperatures preferably not much in excess of 100° centigrade and then adding the soda. The mixture is stirred until a foamy condition occurs, and may then be placed in molds and permitted to cool. When cooled it will be of a permanently elastic sponge-like nature.

A body having the cellular and elastic characteristics of those above-described will, of course, absorb a considerable quantity of sound waves by reason of its porous or cellular structure and by reason of its elasticity and the flexibility of the mass as a whole, as well as of the walls of the cells, the sound waves being transformed into heat energy through the heating of the mass and the friction within the pores.

Other materials, such as felt which is made up of the fibers or hairs found in nature, or on animals, are very definitely limited because of the limitations of the raw material, as to size, length, absorbing power, strength, durability, etc. These have porosity, but the amount of porosity can be controlled only through a very limited extent; it is easily changed through handling and pressure, and does not have the yielding quality of the material which I produce. Another very distinct feature and quality is that my material while highly porous, is a homogeneous mass of one piece, and not merely loosely associated fibers or small particles.

In Figs. 6 and 7, I show a structure composed of crossed strands 10 and 11 which may extend along substantially straight lines in various directions, or may be heterogeneously assembled.

These strands 10 and 11 may be formed of rubber, in which case they can be vulcanized together at their points of intersection to form a homogeneous mass. The vulcanization could be effected in a mold, with the application of heat, in a manner common in the rubber industry.

The strands can also be formed of other material such as asbestos, in case a fire proof body is desired and one which is not subject to decay. The asbestos or other strands of thread-like or ribbon-like form may be glued or cemented together to maintain them in unitary relation. The fibers of Figs. 6 and 7 are preferably manufactured in such form and of such materials as to possess predetermined physical characteristics and they may be of such diameter and spaced such distances apart as will produce a body having pores of a desired size and number.

The material may be made up in the form of units or slabs of convenient size which may be applied to walls, ceilings, or the like, by gluing, nailing or the like, and its flexibility permits it to be closely and accurately applied to curved surfaces, corners, etc., by unskilled workmen, with the assurance that the sound-absorbing capacity of the material when applied will be definitely known in advance, according to the structure of the units. Again, the material is compressible and if a piece is slightly too large for a given piece, it can be compressed therein. Again, it may be stretched somewhat in order to fill a larger space.

When a unit is stretched, to a desired extent, it can be either glued or fastened in such position or, in the case of the porous rubber, it can be stretched by the workmen and held in such position until the heat generated by the stretching action has been dissipated, whereupon the unit will become set in an expanded position.

Also, the units being elastic can be placed in slightly-compressed abutting relation with one another, thus substantially eliminating marked visible lines of division which are usually present between sound-absorbing units of a more rigid nature.

Ordinarily, the elastic bodies will be largely cellular, that is, they will be composed almost entirely of cells divided only by thin walls, instead of being largely solid and containing cells spaced considerable distances apart.

I claim as my invention:—

1. A sound-absorbing body containing cells whose walls are flexible and highly elastic, and of such thinness that they will vibrate under the influence of sound waves, the cells in one portion of the body being of a predetermined average size, and the cells in another portion of the body being of another predetermined average size.

2. A sound-absorbing unit comprising strips of flexible elastic material arranged in crossed relation to form cells.

3. A sound-absorbing unit comprising a plurality of pieces of flexible elastic material arranged in superposed relation, various of the pieces being assembled in non-compact relation to form cells within the unit, the said pieces being of greater length than thickness.

JACOB MAZER.